

# United States Patent Office.

CARL PETRUS ALSING, OF NEW YORK, N. Y.

*Letters Patent No. 98,460, dated January 4, 1870.*

## IMPROVEMENT IN ASPHALT PAVEMENTS.

The Schedule referred to in these Letters Patent and making part of the same

*To all whom it may concern:*

Be it known that I, CARL PETRUS ALSING, of the city, county, and State of New York, have invented a new and useful Improvement in Asphalt Pavements; and I do hereby declare the following to be a full, clear, and exact description of the same.

The nature of my invention consists in a compound for asphalt pavement, composed of asphalt, distilled coal or pine-tar, pulverized flint, pulverized oyster-shells, zinc-white, pulverized bone, and gravel.

To enable others skilled in the art to make and use my improvement, I will proceed to describe its operation.

The ingredients of which the pavement is composed are prepared in two separate apparatus, one to contain the ingredients which are intended to form the lower or bottom layer, and the other apparatus to contain the ingredients forming the upper or top layer of the pavement.

For the bottom layer, may be used coarse asphalt and pine or coal-tar, but for the upper layer, I use a compound of the following ingredients:

Asphalt, thirty-five parts.

Distilled coal or pine-tar, fifteen parts.

Zinc-white, two parts.

Pulverized oyster-shells, two parts.

Pulverized flint, five parts.

Pulverized bone, one part.

Gravel, (well screened,) forty parts.

The ground on which the pavement is to be laid, should be dry, level, and covered with a layer of coarse gravel, and carefully rammed.

One hour after the bottom layer is laid, it is ready

to receive the upper layer, which may be of any desired thickness, according to circumstances.

The upper layer is levelled with a straight-edge, or any other suitable device.

While the layer is still hot and soft, it is covered with a layer of gravel of the size of a pea, and in order to prevent the gravel from being swept off or becoming loose, it may be pressed down and embedded in the compound of which the upper layer of the pavement consists.

The compound of my asphalt pavement is particularly adapted to cover streets, roads in parks, &c., and neither the tread of horses nor the wheels of carriages will produce any injurious effect upon the pavement.

The durability of the composition depends, in a great measure, upon the quality and preparation of the asphalt.

Having thus described my invention,

What I claim as my invention, and desire to secure by Letters Patent, is—

The manufacture or preparation of a compound which is denominated asphalt pavement, of the ingredients, in the proportions, and for the purposes set forth.

In testimony whereof, I have signed my name to this specification, in the presence of two subscribing witnesses.

CARL PETRUS ALSING.

Witnesses:

C. F. CLAUSEN,

A. RUPPERT.